

Patented Nov. 22, 1927.

## UNITED STATES PATENT OFFICE.

ARLIE WILLIAM SCHORGER, OF MADISON, WISCONSIN, ASSIGNOR, BY MESNE ASSIGNMENTS, TO C. F. BURGESS LABORATORIES, INC., OF DOVER, DELAWARE, A CORPORATION OF DELAWARE.

## ROOFING FELT.

No Drawing. Application filed December 20, 1924, Serial No. 757,297. Renewed October 1, 1927.

Manufacturers of asphalt shingles utilize each year an enormous tonnage of felt. The 5 felt is saturated with asphaltic material to serve as the body of the shingle, it being customary to surface one face of the saturated felt with a bituminous material having a high melt point and serving as a binder for slate or other mineral or metal particles which act as the weathering face of the shingle. 10 Such felt must be of considerable strength, for in the ordinary operation of shingle manufacture it is drawn at relatively high speed through a long bath of the hot asphalt. Any tearing of the felt while passing through the bath seriously interrupts the manufacturing operation, for the steps of drying on the looper and the subsequent steps of surfacing with bitumen, sprinkling with slate, and cutting into shingles, are all 15 timed to accommodate continuous passage of the felt through the plant. Any interruption due to breakage of the felt not only shuts down the entire saturating machine and its adjuncts, but is likely to result in 20 considerable loss of material. To avoid these inconveniences, a relatively large percentage of long fibred stock is used in the manufacture of the felt. Clean cotton rags, woolen cloth, waste wool, and the like are 25 relied on to give the necessary tensile strength to the finished felt, even though it may contain some short-fibred stock, such as can be had by beating up old newspapers, and similar semiwaste products.

30 It is the object of the present invention to lessen the cost of felt suitable for use in the manufacture of asphalt shingles by making this felt, in part at least, out of a component of discarded automobile tire casings. Such 35 casings consist, in large measure, of rubber interspersed with cotton fabric. High grade cotton is used for this purpose, and I have found a way of separating it from the rubber without shortening the fibres unduly.

40 The long-fibred stock of high quality thus obtained, with such rubbery components as cling to the fibres, is, I have found, a very excellent material for use in place of the cotton and wool rags heretofore utilized so 45 extensively in the manufacture of roofing felts.

50 The process whereby the desired end is attained may consist of cutting the tire casings into strips about one-half inch width,

and then feeding them into a shredder or 55 disc mill of one of the types now standard in the paper making industry for shredding cooked wood pulp, or chipped wood. The shredding operation, whichever machine is used, serves to break up the rubber into 60 small particles, and in large measure serves to free the cotton fibres from the rubber. Air separation can be used for freeing the mass from the cotton fibres. The fibres so obtained are relatively long and strong, having 65 originally been of very excellent quality, and having been well protected by the rubber against rot and similar attack. Fibres so obtained will ordinarily be accompanied by a certain amount of rubber, because of 70 the previous intimate contact and adhesion between the fabric and the rubber in the tire. This, however, is not a disadvantage, and in my opinion, is a very considerable advantage, when the cotton fibre is to be used 75 in the manufacture of roofing, for this rubber, which may be conceived of as somewhat in the nature of a film on the shredded fibres, acts as a flux to facilitate the subsequent impregnation with asphalt of a felt sheet 80 wherein these cotton fibres are an ingredient.

To incorporate this cotton in the felt, it is only necessary to substitute the cotton fibres for an equivalent amount of cotton rags, wool rags, shoddy, and the like, when 85 the raw material is charged into the beaters at the felt plant.

The proportions in which cotton fibres of old tire casings shall be used in the roofing felt will, in large measure, be governed by 90 commercial considerations, but the greater the percentage of cotton fibre, the stronger will be the felt. Conversely, for an equal strength of felt, a considerably larger percentage of old newspapers and short fibre 95 stock can be charged into the beaters.

The various operations of beating, mixing, felting and drying may be the same as those ordinarily employed in making roofing felt. When such a felt is utilized at a 100 roofing plant, its good qualities quickly become apparent. Not only is it strong and tough, per unit of cost, but the hot asphalt through which it is rapidly passed penetrates quickly through the sheet and gives 105 the desired uniform impregnation, that action being no doubt facilitated by the presence on the fibres of some residue of rubber

from the original tires, that rubber acting much as a flux to bring the asphaltum quickly into intimate contact with the fibres and assisting perhaps also in the penetration of 5 the asphalt into the inner portions of the felt. Such rubber as may remain in the finished sheet-roofing or shingle is not a detriment therein, but on the contrary, is advantageous, particularly because of its intimate 10 contact with and protective action on the long and strong cotton fibres by which the shorter fibres and loading materials are held in place as a coherent sheet.

At the present time old tire casings or 15 shoes have no market value and ordinarily are burned at the garages after they cease to be of value on automobiles. During the war when the price of raw rubber was high a certain amount of work was done on reclaiming old tires for their rubber content, but at the present normal price of raw rubber, there is, I believe, no commercial demand for old tire casings for that purpose. 20

In a companion application, Serial No. 25 757,296 filed December 20, 1924, I have described and claimed a process of making a veneer core out of the rubber content of old tire casings, and when that is done, or when the rubber content is used in any similar manner, the cotton fibre content is in the nature of a by-product. It is an object of the present invention to utilize that by-

product, and in a manner and to an extent that will prevent what is now a large economic waste.

I claim:

1. A roofing felt comprising an appreciable quantity of cotton fibres recovered from old tire casings, and having a small quantity of rubber admixed therewith substantially as 40 described.

2. An asphalt roofing containing cotton fibres with such quantity of rubber as normally will be associated with the fibres when they are obtained from old tire casings by shredding and air separation, substantially as described. 45

3. The method which consists in shredding old tire casings to liberate the fibres of the tire fabric, subjecting the shredded material to an air blast to imperfectly separate the cotton from the rubber, making a roofing felt wherein the cotton so obtained is an essential ingredient, and subsequently saturating said felt with asphaltic material, 50 substantially as described.

4. In the impregnation of a roofing felt with asphaltic material the step which consists in using in the felt stock an appreciable quantity of cotton fibres recovered 60 from old tire casings and having a small quantity of rubber admixed therewith.

In testimony whereof I affix my signature.

ARLIE WILLIAM SCHORGER.